



US007517428B2

(12) **United States Patent**  
**Nun et al.**

(10) **Patent No.:** **US 7,517,428 B2**  
(45) **Date of Patent:** **Apr. 14, 2009**

(54) **PRODUCTION OF SELF-CLEANING SURFACES ON TEXTILE COATINGS**

(75) Inventors: **Edwin Nun**, Billerbeck (DE); **Markus Oles**, Hattingen (DE)

(73) Assignee: **Degussa AG**, Duesseldorf (DE)

(\*) Notice: Subject to any disclaimer, the term of this patent is extended or adjusted under 35 U.S.C. 154(b) by 188 days.

(21) Appl. No.: **10/526,559**

(22) PCT Filed: **Jul. 26, 2003**

(86) PCT No.: **PCT/EP03/08280**

§ 371 (c)(1),  
(2), (4) Date: **Mar. 4, 2005**

(87) PCT Pub. No.: **WO2004/033788**

PCT Pub. Date: **Apr. 22, 2004**

(65) **Prior Publication Data**

US 2006/0128239 A1 Jun. 15, 2006

(30) **Foreign Application Priority Data**

Sep. 13, 2002 (DE) ..... 102 42 560

(51) **Int. Cl.**

**C09J 5/02** (2006.01)  
**B44C 1/165** (2006.01)  
**B44C 1/24** (2006.01)  
**B32B 37/14** (2006.01)  
**B32B 33/00** (2006.01)  
**B44C 1/17** (2006.01)  
**B32B 37/22** (2006.01)

(52) **U.S. Cl.** ..... **156/306.3; 156/230; 156/247; 156/289; 428/40.1; 428/41.8; 428/42.2**

(58) **Field of Classification Search** ..... 156/230, 156/245-247, 289, 325, 329, 334, 306.3; 428/40.1, 41.8, 42.2-42.3

See application file for complete search history.

(56) **References Cited**

**U.S. PATENT DOCUMENTS**

3,650,740 A \* 3/1972 Van Paesschen et al. .... 430/258  
(Continued)

**FOREIGN PATENT DOCUMENTS**

DE 100 22 246 11/2001  
(Continued)

**OTHER PUBLICATIONS**

U.S. Appl. No. 10/526,559, filed Mar. 4, 2005, Nun, et al.  
(Continued)

*Primary Examiner*—Philip C Tucker

*Assistant Examiner*—Sonya Mazumdar

(74) *Attorney, Agent, or Firm*—Oblon, Spivak, McClelland, Maier & Neustadt, P.C.

(57) **ABSTRACT**

The invention relates to a process for producing self-cleaning surfaces on coated textile sheets, by the following steps of the process:

- i.) applying hydrophobic nanostructured particles to a surface of a transfer-medium sheet,
- ii.) applying a coating composition and a textile sheet to those surfaces of the transfer medium to which the hydrophobic nanostructured particles were applied in step i.) of the process,
- iii.) heat treatment of the composite resulting from steps i.) to ii.) of the process, and
- iv.) removing the transfer medium, and also to the coated textile sheets produced by means of the process of the invention, and their use.

**21 Claims, 1 Drawing Sheet**



## U.S. PATENT DOCUMENTS

|                   |         |                       |           |
|-------------------|---------|-----------------------|-----------|
| 5,158,636 A *     | 10/1992 | Groitzsch et al. .... | 156/230   |
| 6,245,188 B1 *    | 6/2001  | Toyoda et al. ....    | 156/344   |
| 6,337,129 B1 *    | 1/2002  | Watanabe et al. ....  | 428/328   |
| 6,638,603 B1 *    | 10/2003 | Kerins et al. ....    | 428/195.1 |
| 6,683,126 B2 *    | 1/2004  | Keller et al. ....    | 524/492   |
| 6,811,856 B2      | 11/2004 | Nun et al.            |           |
| 6,852,389 B2      | 2/2005  | Nun et al.            |           |
| 6,858,284 B2      | 2/2005  | Nun et al.            |           |
| 6,977,094 B2      | 12/2005 | Oles et al.           |           |
| 7,083,828 B2      | 8/2006  | Muller et al.         |           |
| 2002/0148601 A1   | 10/2002 | Roos et al.           |           |
| 2002/0150723 A1   | 10/2002 | Oles et al.           |           |
| 2002/0164443 A1   | 11/2002 | Oles et al.           |           |
| 2002/0192385 A1   | 12/2002 | Jenkner et al.        |           |
| 2003/0013795 A1   | 1/2003  | Nun et al.            |           |
| 2003/0049396 A1   | 3/2003  | Oles et al.           |           |
| 2003/0134086 A1   | 7/2003  | Nun et al.            |           |
| 2003/0147932 A1   | 8/2003  | Nun et al.            |           |
| 2004/0028913 A1   | 2/2004  | Hennige et al.        |           |
| 2004/0154106 A1   | 8/2004  | Oles et al.           |           |
| 2004/0171515 A1 * | 9/2004  | Hamers et al. ....    | 510/504   |
| 2005/0070193 A1   | 3/2005  | Hennige et al.        |           |
| 2005/0084653 A1   | 4/2005  | Nun et al.            |           |
| 2005/0103457 A1   | 5/2005  | Nun et al.            |           |
| 2005/0112326 A1   | 5/2005  | Nun et al.            |           |
| 2005/0118433 A1   | 6/2005  | Oles et al.           |           |
| 2005/0163951 A1   | 7/2005  | Oles et al.           |           |

|                 |         |             |
|-----------------|---------|-------------|
| 2005/0167877 A1 | 8/2005  | Nun et al.  |
| 2005/0205830 A1 | 9/2005  | Oles et al. |
| 2005/0208269 A1 | 9/2005  | Nun et al.  |
| 2005/0227045 A1 | 10/2005 | Oles et al. |
| 2005/0253302 A1 | 11/2005 | Nun et al.  |
| 2006/0128239 A1 | 6/2006  | Nun et al.  |

## FOREIGN PATENT DOCUMENTS

|    |              |         |
|----|--------------|---------|
| DE | 101 35 157   | 2/2003  |
| EP | 1153987 A2 * | 11/2001 |
| JP | 5411577 A *  | 9/1979  |

## OTHER PUBLICATIONS

|                                                                 |
|-----------------------------------------------------------------|
| U.S. Appl. No. 10/551,841, filed Oct. 3, 2005, Nun, et al.      |
| U.S. Appl. No. 10/556,092, filed Nov. 9, 2005, Oles, et al.     |
| U.S. Appl. No. 11/312,469, filed Dec. 21, 2005, Nun, et al.     |
| U.S. Appl. No. 11/312,340, filed Dec. 21, 2005, Hennige, et al. |
| U.S. Appl. No. 10/546,979, filed Aug. 26, 2005, Nun, et al.     |
| U.S. Appl. No. 11/321,285, filed Dec. 21, 2005, Oles, et al.    |
| U.S. Appl. No. 11/312,557, filed Dec. 21, 2005, Oles, et al.    |
| U.S. Appl. No. 10/111,407, filed May 6, 2002, Oles, et al.      |
| U.S. Appl. No. 10/527,641, filed Mar. 14, 2005, Nun, et al.     |
| U.S. Appl. No. 09/241,077, filed Feb. 1, 1999, Peters, et al.   |
| U.S. Appl. No. 10/575,268, filed Apr. 11, 2006, Hennige, et al. |
| U.S. Appl. No. 10/588,952, filed Aug. 10, 2006, Nun, et al.     |
| U.S. Appl. No. 11/572,548, filed Jan. 23, 2007, Nun, et al.     |

\* cited by examiner



Fig. 1

## 1

## PRODUCTION OF SELF-CLEANING SURFACES ON TEXTILE COATINGS

## CROSS-REFERENCES TO RELATED APPLICATIONS

This application is a national stage application of International Patent Application No. PCT/EP03/08280, filed on Jul. 26, 2003, and claims priority to German Patent Application No. 102 42 560.4, filed on Sep. 13, 2002, both of which are incorporated herein by reference in their entirieties.

The invention relates to a process for producing self-cleaning surfaces on coated textile sheets, and also to the coated textile sheets produced by means of the process of the invention, and to their use.

Various processes for treating surfaces to give these surfaces dirt- and water-repellent properties are known from surface technology. For example, it is known that if a surface is to have good self-cleaning properties it has to have a certain roughness, as well as hydrophobic properties. A suitable combination of structure and hydrophobic properties permits even small amounts of moving water to entrain dirt particles which adhere to the surface and to clean the surface (WO 96/04123, U.S. Pat. No. 3,354,022, C. Neinhuis, W. Barthlott, Annals of Botany 79 (1997), 667).

As early as in 1982, A. A. Abramson in *Chimia i Shisn russ.* 11, 38 described the run-off of water droplets on hydrophobic surfaces, even at very small angles of inclination, especially if the surfaces have structuring, but without self-cleaning being acknowledged, and this description was also provided in Japanese Patent Application JP 07328532 A, in 1994.

The prior art of EP 0 933 388 in relation to self-cleaning surfaces requires an aspect ratio >1 and a surface energy of less than 20 mN/m for these self-cleaning surfaces, the aspect ratio being defined here as the quotient which is the ratio between the average height of the structure and its average width. The abovementioned criteria are to be found in the natural world, for example in lotus leaves. The lotus plant has a leaf surface formed from a hydrophobic waxy material and having elevations separated from one another by up to a few  $\mu\text{m}$ . Water droplets substantially come into contact only with the peaks of the elevations. There are many descriptions in the literature of water-repellent surfaces of this type. A relevant example here is an article in *Langmuir* 16 (2000), 5754, by Masashi Miwa et al., describing the increase in contact angle and roll-off angle with increasing structuring of artificial surfaces formed from boehmite, applied to a spin-coated layer and then calcined.

Swiss Patent 268258 describes a process which generates structured surfaces by applying powders, such as kaolin, talc, clay, or silica gel. Oils and resins based on organosilicon compounds are used to secure the powders to the surface. An adhesion promoter is also used in the Offenlegungsschrift DE 100 22 246 A1.

It is known that hydrophobic materials, such as perfluorinated polymers, can be used to produce hydrophobic surfaces. DE 197 15 906 A1 states that perfluorinated polymers, such as polytetrafluoroethylene or copolymers of polytetrafluoroethylene with perfluoroalkyl vinyl ethers, can generate hydrophobic surfaces which have structuring and have low adhesion to snow and ice. JP 11171592 describes a water-repellent product and its production, the dirt-repellent surface being produced by applying, to the surface to be treated, a film which comprises fine particles of metal oxide and comprises the hydrolyzate of a metal alkoxide or of a metal chelate. To consolidate this film, the substrate to which the film has been applied has to be sintered at temperatures above 400° C. This

## 2

process is therefore usable only for substrates which can be heated to temperatures above 400° C. without damage or warping.

In recent times, attempts have also been made to provide self-cleaning surfaces on textiles. It has been found that self-cleaning surfaces can be produced, for example by applying hydrophobic, fumed silicas to textiles. These hydrophobic, fumed silicas are bonded into the polymer matrix of the textile fiber with the action of a solvent.

10 In DE 101 18 348, polymer fibers with self-cleaning properties are described, their self-cleaning surface being obtained by

the action of a solvent which comprises structure-forming particles,

15 solvation of the surface of the polymer fibers by this solvent, adhesion of the structure-forming particles to the solvated surface, and removal of the solvent.

20 A disadvantage of this process is that when the polymer fibers are processed (spinning, knitting, etc.) the structure-forming particles, and therefore the structure responsible for the self-cleaning surface, can become damaged or sometimes even be lost entirely, with the result that the self-cleaning effect is likewise lost.

25 DE 101 18 346 describes textile sheets with self-cleaning and water-repellent surface, composed of at least one synthetic and/or natural textile base material A and of an artificial, at least to some extent hydrophobic, surface with elevations and depressions made from particles which have been securely bonded to the base material A without adhesives, resins, or coatings. These elevations and depressions are obtained by treating the base material A with at least one solvent which comprises the undissolved particles, and

30 removing the solvent, whereupon at least some of the particles become securely bonded to the surface of the base material A. However, the disadvantage of this process is the very complicated finishing of the textile surfaces. This process requires precise matching of the solvent to the base

35 material of the textiles. However, in clothing there are generally mixed fabrics present, further complicating this matching process. If the matching of the solvents is not precise, the result can be irreparable damage to parts of the clothing. These surfaces therefore have to be treated prior to tailoring.

40 DE 101 35 157 describes a process for the coating of textiles during a dry-cleaning procedure, in which structure-forming particles are added to the cleaning agent. The cleaning agents proposed are organic solvents which are relatively hazardous to health, e.g. trichloroethylene or perchloroethylene, and the use of these solvents leads to mechanical anchoring of the particles to the structure of the textiles.

45 The conventional processes for producing self-cleaning surfaces are complicated and many of them have limited use. For example, embossing techniques are inflexible with

50 respect to the application of structures to variously shaped three-dimensional bodies or sheets with or without fabric inserts. There is no suitable current technology for producing flat, large-surface-area web product, particularly for web product with a fabric insert. Processes in which structure-

55 forming particles are applied to surfaces by means of a carrier—for example an adhesive or binder—have the disadvantage that the resultant surfaces are composed of various combinations of material which, for example, have different coefficients of thermal expansion, and this can lead to damage to the surface. Severe flexing or creasing can lead to cracking in these surfaces made from various combinations of material, and for this reason products produced in this way are not

very suitable as protective films or tarpaulins, since these should at least to some extent adapt to the contours of the articles to be provided with protective cover. Hitherto, there has been no way to equip coatings for textile sheets with permanent water-repellent or indeed self-cleaning properties.

It was therefore an object of the present invention to provide a process for producing self-cleaning surfaces on coated textile sheets, where the resultant coated textile sheets can be flexed or creased with minimum cracking. The production of coated textile sheets is therefore intended to require no use of adhesives, binders, adhesion promoters, or other additional materials, other than the coating itself, thus retaining the flexibility of the coated textile sheet. A further intention is to avoid the use of any embossing technique in relation to the production of the self-cleaning surfaces on coated textile sheets, since these techniques are still at an early stage of their development and would require high capital expenditure. A further intention is that the method for applying the particles to the surface of the coated textile sheet does not involve a complicated downstream step of the process, e.g. application of the particles in a process which temporarily solvates the surface of the coated textile sheet with the aid of a solvent in order to achieve adhesion of the particles to the surface. A further object of this invention was therefore to integrate the step of the process which applies the particles into a prior-art process. A further object of the invention was to provide long-term anchoring of the particles to or within the surface of the coated textile sheet, thus making the self-cleaning surfaces longlasting.

Surprisingly, it has been found that coated textile sheets with a self-cleaning surface can be produced by, in a first step of the process, applying the particles to at least one surface of a transfer-medium sheet, and, in a further step of the process, applying a coating composition and a textile sheet to that surface of the transfer medium to which the particles were applied in the first step of the process. This is followed by heat treatment of the resultant composite and the removal of the transfer medium. The process of the invention can produce coated textile sheets which have a long-term self-cleaning surface. A sufficient number and density of the hydrophobic nanostructured particles can be bonded firmly into or onto the surface of the coating composition. This is particularly surprising since the coating composition is generally hydrophilic, and binding of the hydrophobic particles was unexpected.

#### BRIEF DESCRIPTION OF THE DRAWING

FIG. 1 shows a particle with fine structure embedded in the surface of a coated textile sheet according to the claimed invention.

The present invention provides a process for producing self-cleaning surfaces on coated textile sheets, where the process has the following steps of:

- i.) applying hydrophobic nanostructured particles to a surface of a transfer-medium sheet,
- ii.) applying a coating composition and a textile sheet to those surfaces of the transfer medium to which the hydrophobic nanostructured particles were applied in step i.) of the process,
- iii.) heat treatment of the composite resulting from steps i.) to ii.) of the process, and
- iv.) removing the transfer medium.

The present invention also provides coated textile sheets which have hydrophobic nanostructured particles on the coating surface, and their use for the production of clothing, of technical textiles, and of fabrics for textile buildings.

The process of the invention provides access to coated textile sheets with self-cleaning properties, which may have (fabric) inserts. This process produces the self-cleaning properties without further application of material, such as a binder or adhesive—other than the particles themselves. Advantageously, the process of the invention can avoid the use of a downstream finishing process on the coated textile sheets. This method can produce coated textile sheets with self-cleaning properties which again, when compared with the 10 coated textile sheets of the prior art, have good flexibility when creased or flexed. A particularly advantageous feature has proven to be that the areas of textile sheets for which the process of the invention can be used can be almost as large as desired. The process of the invention can moreover be used to 15 equip both sides of the coated textile sheet with self-cleaning properties, for example, through subsequent reverse-side coating. The coated textile sheets of the invention with surfaces which have self-cleaning properties and have surface structures with elevations feature coatings which are preferably synthetic-polymer surfaces into which the particles have 20 been directly anchored, and not bound by way of carrier systems or the like.

The process for producing self-cleaning surfaces on coated textile sheets has the following steps:

- 25 i.) applying hydrophobic nanostructured particles to a surface of a transfer-medium sheet,
- ii.) applying a coating composition and a textile sheet to those surfaces of the transfer medium to which the hydrophobic nanostructured particles were applied in step i.) of the process,
- 30 iii.) heat treatment of the composite resulting from steps i.) to ii.) of the process, and
- iv.) removing the transfer medium.

In step i.) of the process of the invention, hydrophobic nanostructured particles are applied to a surface of a transfer-medium sheet. The surface of the transfer medium preferably has hydrophobic properties. As the level of hydrophobic properties of the transfer medium reduces, uniform distribution of the nanostructured hydrophobic particles becomes 35 increasingly difficult, as therefore also does uniform transfer to the coating of the textile sheet, and this is almost impossible in the case of hydrophilic transfer media. A preferred transfer medium used is a lamination paper, particular preferably a siliconized or otherwise hydrophobicized lamination paper.

40 Hydrophobic nanostructured particles which may be used in step i.) of the process of the invention are those which comprise at least one material selected from minerals, aluminum oxide, silicates, hydrophobically modified silicas, metal oxides, mixed oxides, metal powders, pigments, and polymers. The particles may particularly preferably be silicates, doped silicates, minerals, metal oxides, aluminum oxide, precipitated silicas (Sipernat® grades), fumed silicas (Aerosil® grades), or pulverulent polymers, e.g. spray-dried and agglomerated emulsions or cryogenically milled PTFE. The 45 hydrophobic particles used are particularly preferably hydrophobicized silicas.

In step i.) of the process of the invention, it is preferable to use hydrophobic nanostructured particles which have an average diameter of from 0.01 to 100 µm, particularly preferably 50 from 0.02 to 50 µm, and very particularly preferably from 0.05 to 30 µm. However, other suitable particles are those accreted from primary particles in the suspension medium to give agglomerates or aggregates whose size is from 0.02 to 100 µm.

55 In step i.) of the process of the invention, it can be advantageous for the hydrophobic nanostructured particles used to have a structured surface. It is preferable to use particles

## 5

whose surface has an irregular fine structure in the nanometer range, i.e. in the range from 1 to 1000 nm, preferably from 2 to 750 nm, and very particularly preferably from 10 to 100 nm. Fine structures are structures which have elevations, peaks, crevices, ridges, fissures, undercuts, notches, and/or holes with the specified dimensions and within the specified scope. These nanostructured particles preferably comprise at least one compound selected from fumed silica, fumed mixed oxides, and oxides, such as titanium dioxide or zirconium dioxide, precipitated silicas, aluminum oxide, silicon dioxide, and pulverulent polymers.

The hydrophobic properties of the particles used in step i.) of the process of the invention may be inherently present by virtue of the material used for the particles, for example as is the case with polytetrafluoroethylene (PTFE). However, it is also possible to use hydrophobic particles which have hydrophobic properties after suitable treatment, e.g. particles treated with at least one compound from the group of the alkylsilanes, the fluoroalkylsilanes, and the disilazanes. Particularly suitable particles are hydrophobicized fumed silicas, known as Aerosils®. Examples of hydrophobic particles are Aerosil® VPR 411, Aerosil® VP LE 8241, and Aerosil® R 8200. Examples of particles which can be hydrophobicized by treatment with perfluoroalkylsilane followed by heat-conditioning are Aeroperl 90/30®, Sipernat silica 350®, aluminum oxide C®, zirconium silicate, and vanadium-doped or VP Aeroperl P 25/20®.

The hydrophobic nanostructured particles are preferably applied in the form of a suspension to the transfer medium, examples for methods for this being spray-application or doctoring, in particular by means of a spreader-doctor. The suspension preferably comprises from 1 to 20% by weight, with preference from 2 to 15% by weight, and very particularly preferably from 3 to 12% by weight, of particles, based on the suspension.

The organic solvent used preferably comprises acetone, tetrahydrofuran, butyl acetate, toluene, dimethylformamide, acetonitrile, dimethyl sulfoxide, decalin, or an alcohol liquid at room temperature, in particular methanol, ethanol, n-propanol, or isopropanol. The alcohol used is very particularly preferably ethanol. However, it can also be advantageous for the suspension used to comprise a mixture of these organic solvents.

Once the hydrophobic nanostructured particles have been applied, the suspension medium is advantageously removed from the particle-containing suspension by vaporization or evaporation, and this vaporization or evaporation may be accelerated by using elevated temperatures or using subatmospheric pressure or vacuum.

In step ii.) of the process of the invention, a coating composition and the textile sheet are applied to those surfaces of the transfer medium to which the hydrophobic nanostructured particles were applied in step i.) of the process.

The coating composition preferably comprises at least one polymer selected from polyvinyl chloride, polyurethane, acrylonitrile-butadiene-styrene terpolymer (ABS), polychloroprene, in the form of a suspension, alone or together with a reactive monomer mixture which after a reaction forms at least one of the abovementioned polymers, the material here preferably being a reactive paste, particularly preferably a commercial product with good suitability for the particular use, e.g. coating compositions from the product lines Impraperm® (Bayer AG), Impranil® (Bayer AG), Baystal® (Polymer Latex GmbH), Plextol® (Polymer Latex GmbH), Liopur® (Synthopol Chemie), Larithane® and Laripur® (both Novotex Italy). The coating composition preferably has hydrophilic properties.

## 6

In a particular embodiment of the process of the invention, in step ii.) of the process, the coating composition is first applied to those surfaces of the transfer medium to which the hydrophobic nanostructured particles were applied in step i.) of the process, and then the textile sheet is applied to this coating composition.

In another particular embodiment of the process of the invention, in step ii.) of the process, the coating composition is first applied to the surfaces of the textile sheet, and then this composite is applied to those surfaces of the transfer medium to which the hydrophobic nanostructured particles were applied in step i.) of the process, the location of the coating composition being between the transfer medium, with its particles, and the textile sheet.

In both of the embodiments mentioned of the process of the invention, the coating composition may be applied by means of processes familiar to the skilled worker. The coating composition is preferably applied by means of a roller-coating method to that surface of the transfer medium to which the particles have previously been applied in step i.) of the process, or, respectively, to the textile sheet.

Step iii.) of the process of the invention heat-treats the composite resulting from steps i.) to ii.) of the process. This step of the process of the invention preferably serves to cure the coating composition.

In step iv.) of the process, the transfer medium is preferably peeled away from the coating composition and is then wound up. The transfer medium can thus be used two or more times, preferably from 2 to 15 times, for this process of the invention. In order to ensure that the coating composition applied assumes a uniform lotus effect during the curing process, renewal is preferably required according to the invention on each subsequent occasion of use.

In one particular embodiment of the process of the invention, it is also possible for the coating of a second surface to take place in a downstream step of the process, e.g. coating of the reverse side of the textile sheet. For this, steps i.) to iv.) of the process are carried out for the reverse-side surface of the textile sheet previously single-surface coated by the method of the invention.

This invention further provides coated textile sheets which have hydrophobic nanostructured particles on at least one coating surface, these coated textile sheets preferably being produced by means of the process of the invention.

These coated textile sheets of the invention preferably have, on or in their surface, hydrophobic nanostructured particles which comprise at least one material selected from minerals, aluminum oxide, silicates, silicas, preferably hydrophobically modified silicas, metal oxides, mixed oxides, metal powders, pigments, and polymers. The particles may particularly preferably be silicates, doped silicates, minerals, metal oxides, aluminum oxide, precipitated silicas, or fumed silicas (Aerosil® grades) or pulverulent polymers, e.g. spray-dried and agglomerated emulsions, or cryogenically milled PTFE. The coated textile sheets particularly preferably comprise hydrophobic nanostructured particles which are silicas.

The coated textile sheets of the invention preferably comprise hydrophobic nanostructured particles which have an average diameter of from 0.01 to 100 µm, particularly preferably from 0.02 to 50 µm, and very particularly preferably from 0.05 to 30 µm. They may also comprise particles accreted from primary particles in the suspension medium to give agglomerates or aggregates whose size is from 0.02 to 100 µm.

It can be advantageous for the particles of the coated textile sheets of the invention to have a structured surface. The

surface of the particles preferably has an irregular fine structure in the nanometer range, i.e. in the range from 1 to 1000 nm, preferably from 2 to 750 nm, and very particularly preferably from 10 to 100 nm. Fine structures are structures which have elevations, peaks, crevices, ridges, fissures, undercuts, notches, and/or holes with the specified dimensions and within the specified scope. These nanostructured particles preferably comprise at least one compound selected from fumed silica and fumed oxides, such as titanium dioxide or zirconium dioxide, or from mixed oxides, precipitated silicas, aluminum oxide, silicon dioxide, and pulverulent polymers.

The hydrophobic properties of the particles of the coated textile sheets of the invention may be inherently present by virtue of the material used for the particles, for example as is the case with polytetrafluoroethylene (PTFE). However, the coated textile sheets of the invention may also comprise hydrophobic particles which have hydrophobic properties after suitable treatment, e.g. particles treated with at least one compound from the group of the alkylsilanes, the fluoroalkylsilanes, and the disilazanes. Particularly suitable particles are hydrophobicized fumed silicas, known as Aerosils®. Examples of hydrophobic particles are Aerosil® VPR 411, Aerosil® VP LE 8241, and Aerosil® R 8200. Examples of particles which can be hydrophobicized by treatment with perfluoroalkylsilane followed by heat-conditioning are Aeroperl 90/30®, Sipermat silica 350®, aluminum oxide C®, zirconium silicate, and vanadium-doped or VP Aeroperl P 25/20®.

The surfaces of the coated textile sheets of the invention preferably have a layer with elevations which are formed by the particles themselves, with an average height of from 0.02 to 25 µm and with a maximum separation of 25 µm, preferably with an average height of from 0.05 to 10 µm and/or with a maximum separation of 10 µm, and very particularly preferably with an average height of from 0.03 to 4 µm, and/or with a maximum separation of 4 µm. The surfaces of the coated textile sheets of the invention very particularly preferably have elevations with an average height of from 0.05 to 1 µm and with a maximum separation of 1 µm. For the purposes of the present invention, the separation of the elevations is the separation of the highest elevation of an elevation represented by a particle from the most adjacent highest elevation represented by another directly neighboring particle. If an elevation has the form of a cone, the peak of the cone is the highest elevation of the elevation. If the elevation is a rectangular parallelepiped, the uppermost surface of the rectangular parallelepiped is the highest elevation of the elevation.

The wetting of solids, and therefore the self-cleaning property, may be described by using the contact angle made by a water droplet with the surface. A contact angle of 0° here implies complete wetting of the surface. The static contact angle is generally measured using devices which determine the contact angle optically. The static contact angles measured on smooth hydrophobic surfaces are usually smaller than 125°. The present surfaces of the coated textile sheets of the invention with self-cleaning surfaces have static contact angles preferably greater than 130°, with preference greater than 140°, and very particularly preferably greater than 145°. It has been found, furthermore, that a surface has particularly good self-cleaning properties only when it exhibits a difference of not more than 10° between advancing and receding angle, and for this reason the surfaces of the coated textile sheets of the invention preferably have a difference less than 10°, with preference less than 7°, and very particularly preferably less than 6°, between advancing and receding angle. To determine the advancing angle, a water droplet is placed on

the surface by means of a cannula and the droplet is enlarged on the surface by adding water through the cannula. During enlargement, the margin of the droplet glides over the surface, and the contact angle is determined as the advancing angle.

5 The receding angle is measured on the same droplet, but water is removed from the droplet through the cannula, and the contact angle is measured during reduction of the size of the droplet. The difference between the two angles is termed hysteresis. The smaller the difference, the smaller the interaction of the water droplet with the surface of the substrate, and therefore the better the self-cleaning effect.

10 The aspect ratio of the elevations formed by the particles themselves on the surfaces of the coated textile sheets of the invention with self-cleaning properties is preferably greater than 0.15. The elevations formed by the particles themselves preferably have an aspect ratio of 0.3 to 0.9, particularly preferably from 0.5 to 0.8. The aspect ratio is defined here as the quotient which is the ratio of the maximum height to the maximum width of the structure of the elevations.

15 20 The surface of particularly preferred coated textile sheets of the invention comprises particles with an irregular, slightly fissured fine structure, the particles preferably having elevations whose aspect ratio in the fine structures is greater than 1, particularly preferably greater than 1.5. The aspect ratio is in turn defined as the quotient which is the ratio of the maximum height to the maximum width of the elevation. FIG. 1 illustrates diagrammatically the difference between the elevations formed by the particles and the elevations formed by the fine structure. The figure shows the surface of a textile sheet

25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9

textile sheet. In another embodiment of the coated textile sheet, the hydrophobic nanostructured particles are present only in some regions of all of the sides of the surface, but preferably only on one side of the surface.

The coated textile sheets of the invention may be used for the production of clothing, in particular for the production of protective clothing, rainwear, and high-visibility safety clothing, or for technical textiles, in particular for the production of protective tarpaulins, tenting, protective covers, truck tarpaulins, or fabrics for textile buildings, and in particular for the production of sun-screening covers, such as awnings, sunshades, parasols.

Examples of uses of the coated textile sheets of the invention are the production of textiles for personal clothing, for the production of textiles for protective clothing, and materials for textile buildings. These coated textile sheets of the invention may, for example, be applied to buildings or vehicles so that these likewise have self-cleaning properties. However, other examples of uses of the coated textile sheets of the invention are found in the textile building sector, for the production of awnings or for sun-screening covers, or else for protective tarpaulins, truck tarpaulins, tenting, or protective coverings. The abovementioned tarpaulins are therefore also provided by the present invention. Preferred uses of the coated textile sheets of the invention are outer rainwear and safety clothing colored for high visibility.

The examples below are intended to provide further illustration of the process of the invention, and also of the coated textile sheets of the invention, but there is no intention that the invention be restricted to this embodiment.

#### EXAMPLE 1

A 10% strength by weight suspension of Aerosil® VP LE 8241 was prepared in a solvent. This suspension was applied by means of a pump spray to a kraft lamination paper (from SCA Flex Pack Papers GmbH, Mannheim). The amount of Aerosil on the pretreated lamination paper was 5 g/m<sup>2</sup>. After evaporation of the solvent at room temperature, LARITHANE AL 227—an aliphatic polyurethane dispersion from Novotex Italy—was applied to the pretreated lamination paper by means of a film-drawing doctor, using a layer thickness of 50 µm. A tricot fabric composed of a nylon fabric (DECOTEX from IBENA Textilwerke Beckmann GmbH) was laminated into the surface of the polyurethane coating before it had fully dried. The polyurethane coating was hot-cured at a temperature of 150° C. for 2 minutes, and then the lamination paper was removed.

TABLE 1

| Experimental parameters and results of characterization for Example 1 |                    |                 |                |
|-----------------------------------------------------------------------|--------------------|-----------------|----------------|
| Experiment                                                            | Solvent            | Advancing angle | Receding angle |
| 1.1                                                                   | Ethanol, denatured | 152.3°          | 149.6°         |
| 1.2                                                                   | Isopropanol, pure  | 149.9°          | 149.0°         |

#### EXAMPLE 2

A 10% strength by weight suspension of Aerosil® VP LE 8241 was prepared in denatured ethanol. This suspension was applied by means of a pump spray to a kraft lamination paper (from SCA Flex Pack Papers GmbH, Mannheim). The

amount of Aerosil on the pretreated lamination paper was 5 g/m<sup>2</sup>. After evaporation of the solvent at room temperature, a polyurethane dispersion as in Table 2 was applied to the pretreated lamination paper by means of a film-drawing doctor, using a layer thickness of 50 µm. A tricot fabric composed of a nylon fabric (DECOTEX from IBENA Textilwerke Beckmann GmbH) was laminated into the surface of the polyurethane coating before it had fully dried. The polyurethane coating was hot-cured at a temperature of 150° C. for 2 minutes, and then the lamination paper was removed.

TABLE 2

| Experiment | Polyurethane dispersion                                    |           |
|------------|------------------------------------------------------------|-----------|
|            | Name                                                       | Type      |
| 2.1/3.1    | Larithane AL 227                                           | Aliphatic |
| 2.2/3.2    | Laripur SH1020<br>in methyl ethyl ketone/dimethylformamide |           |
| 2.3/3.3    | Impranil ENB-03                                            | Aromatic  |
| 2.4/3.4    | Larithane MA 80                                            | Aromatic  |

The coated textile sheets were initially characterized visually, the result recorded being +++ for all four experiments. +++ means that there is almost complete water droplet formation. The roll-off angle is below 10°.

#### EXAMPLE 3

A 1.3% strength by weight suspension of Aerosil® VP LE 8241 was prepared in denatured ethanol. This suspension was applied by means of a propellant spray comprising a propane/butane mixture as propellant to a kraft lamination paper (from SCA Flex Pack Papers GmbH, Mannheim). The amount of Aerosil on the pretreated lamination paper was 5 g/m<sup>2</sup>. After evaporation of the solvent at room temperature, a polyurethane dispersion as in Table 2 was applied to the pretreated lamination paper by means of a film-drawing doctor, using a layer thickness of 50 µm. A tricot fabric composed of a nylon fabric (DECOTEX from IBENA Textilwerke Beckmann GmbH) was laminated into the surface of the polyurethane coating before it had fully dried. The polyurethane coating was hot-cured at a temperature of 150° C. for 2 minutes, and then the lamination paper was removed.

The coated textile sheets were first characterized visually, the recorded result being +++ for all four experiments. +++ means almost complete water droplet formation. The roll-off angle is below 10°.

What is claimed is:

1. A process for producing a self-cleaning surface on a coated textile sheet, said process comprising:
  - i) applying a plurality of hydrophobic particles having a nanostructured surface to a surface of a transfer-medium sheet,
  - ii) applying a coating composition and a textile sheet to said surface of said transfer-medium sheet to which said plurality of hydrophobic particles having a nanostructured surface were applied to obtain a composite,
  - iii) heat treating said composite, and
  - iv) removing said transfer-medium sheet from the composite and transferring the hydrophobic particles to the textile sheet to form the coated textile sheet having a self-cleaning surface comprising the hydrophobic particles having a nanostructured surface, wherein the process for producing a self-cleaning surface on a coated textile

## 11

- sheet is carried out without the use of any adhesive, binder, or adhesion promoter.
2. The process as claimed in claim 1, wherein said transfer-medium sheet has a hydrophobic surface.
3. The process as claimed in claim 2, wherein said transfer-medium sheet is a lamination paper.
4. The process as claimed in claim 1, wherein said particles have an average diameter of from 0.01 to 100  $\mu\text{m}$ .
5. The process as claimed in claim 1, wherein said particles have an average diameter of from 0.02 to 50  $\mu\text{m}$ .
6. The process as claimed in claim 1, wherein said particles are selected from the group consisting of minerals, aluminum oxide, silicates, hydrophobically modified silicas, metal oxides, mixed oxides, metal powders, pigments, polymers, and mixtures thereof.
7. The process as claimed in claim 1, wherein said particles have hydrophobic properties after treatment with at least one compound selected from the group consisting of alkylsilanes, fluoroalkylsilanes, and disilazanes.
8. The process as claimed in claim 1, wherein said coating composition has hydrophilic properties.
9. The process as claimed in claim 1, wherein said coating composition comprises polyvinyl chloride, acrylonitrile-butadiene-styrene terpolymer (ABS), polychloroprene, or polyurethane.
10. The process as claimed in claim 1, wherein in said applying, said coating composition is first applied to said surface of said transfer-medium sheet to which said hydrophobic particles were applied, and then said textile sheet is applied to said coating composition.
11. The process as claimed in claim 1, wherein in said applying, said coating composition is first applied to said surface of said textile sheet, and then said composite is applied to said surface of said transfer-medium sheet to which said hydrophobic particles were applied the location of said

## 12

- coating composition being between said transfer medium sheet, with said particles, and said textile sheet.
12. A method for the production of a clothing, a technical textile, or a fabric for a textile building, said method comprising:
- 5 producing said clothing, said technical textile or said fabric for a textile building with a coated textile sheet having a self-cleaning surface produced by said process as claimed in claim 1.
- 10 13. The method as claimed in claim 12, wherein said clothing is produced and said clothing is a rainwear or a safety clothing with high visibility.
- 15 14. The method as claimed in claim 12, wherein said technical textile is produced and said technical textile is a sun-screening cover.
- 15 15. The method as claimed in claim 12, wherein said fabric for textile building is produced and said fabric is a protective tarpaulin, a tenting, a truck tarpaulin, or another protective covering.
- 20 16. The process as claimed in claim 1, wherein the hydrophobic particles have an irregular fine nanostructured surface in the nanometer range.
- 25 17. The process as claimed in claim 1, wherein the hydrophobic particles have an irregular fine nanostructured surface with features in the range of from 1 to 1,000 nm.
18. The process as claimed in claim 1, wherein the hydrophobic particles have an irregular fine nanostructured surface with features in the range of from 10 to 100 nm.
- 30 19. The process as claimed in claim 1, wherein the process is carried out without an embossing technique.
- 20 20. The process as claimed in claim 1, which is carried out without any solvation of the surface of the coated textile sheet.
- 35 21. The process as claimed in claim 1, wherein the hydrophobic particles have an average diameter of from 30 to 100  $\mu\text{m}$ .

\* \* \* \* \*